

April 13, 1948.

F. R. HENSEL ET AL

2,439,570

ELECTRIC CONTACT

Filed Nov. 10, 1942

Fig. 1



Fig. 3



Fig. 5



Fig. 2



Fig. 4



Fig. 6



Fig. 7



Fig. 10



Fig. 8



Fig. 11



Fig. 9



BY

Robbin - Carlson

ATTORNEYS

## UNITED STATES PATENT OFFICE

2,439,570

## ELECTRIC CONTACT

Franz R. Hensel, Earl I. Larsen, and Earl F. Swazy, Indianapolis, Ind., assignors to P. R. Mallory & Co., Inc., Indianapolis, Ind., a corporation of Delaware

Application November 10, 1942, Serial No. 465,100

3 Claims. (Cl. 75—136)

1

This invention relates to electric contacts.

The present application is related to prior filed co-pending application Serial No. 341,960, filed June 22, 1940, now Patent 2,313,070, granted March 9, 1943.

An object of the invention is to improve electric contacts.

Another object is to provide an abrasion resistant electric contact.

Other objects of the invention will be apparent from the description and claims.

In the drawings

Figure 1 is a face view of an electric contact embodying features of the invention;

Figure 2 is a side view of the contact and the backing therefor;

Figures 3 and 4 are face and side views, respectively, of a contact suited for resistance welding to a backing;

Figures 5 and 6 show another contact suitable for resistance or projection welding;

Figures 7, 8 and 9 are face view, side view and section of another form of contact suited for resistance welding to a backing; and

Figures 10 and 11 are end and side views of a screw type contact assembly.

Recently some uses for electric contacts have been developed where contact materials of the prior art have failed to perform satisfactorily. One application has arisen in connection with airplane engines where the engine vibrations produce a constant "scrubbing" or rotary action of the contacts against each other while they are closed. The abrasive action accompanying the mechanical rubbing between the contacts when they are closed appears to grind off some of the contact metal at the surfaces in a powder form. This powder, perhaps aided in some cases by the presence of oil or moisture, produces a high resistance material between the contacts and raises the contact resistance to an excessively high value in a relatively short time. Tungsten contacts have been tried for this use but have proven unsatisfactory because of the development of this high contact resistance.

We have found that a contact formed of at least 70% of a refractory metal carbide, together with cobalt and silver, will produce a highly satisfactory contact and one which will retain a low contact resistance under the above conditions for an extended period of time. The contact material does not appear to disintegrate to any substantial extent at the surface and hence produces very little loose powder which can result in a high resistance layer.

2

According to the present invention, the material forming the electric contacts will fall within the following range of contact compositions:

|                                                                                                                                                                                                   | Per cent     |
|---------------------------------------------------------------------------------------------------------------------------------------------------------------------------------------------------|--------------|
| Refractory metal carbide selected from the group consisting of tungsten carbide molybdenum carbide, titanium carbide, zirconium carbide, vanadium carbide, columbium carbide and tantalum carbide | 70 to 98     |
| Cobalt                                                                                                                                                                                            | 0.25 to 20   |
| Silver                                                                                                                                                                                            | 0.25 to 24.9 |

The term, "silver" is intended to include pure silver and high silver alloys, such as coin silver and sterling silver. The principal additive metals in the case of silver base alloys are copper, gold, silicon, nickel, manganese, tin, indium, platinum and palladium.

The preferred refractory carbide is tungsten carbide. Either one or both of the tungsten carbides may be used, the preferred one being WC.

Within the above permissible range of compositions, the following preferred ranges may be mentioned:

|                          | Per cent  |
|--------------------------|-----------|
| (A)                      |           |
| Refractory metal carbide | 85 to 95  |
| Cobalt                   | 2 to 10   |
| Silver                   | 5 to 5    |
| (B)                      |           |
| Tungsten carbide         | 87 to 93  |
| Cobalt                   | 6 to 10   |
| Silver                   | 1 to 3    |
| (C)                      |           |
| Refractory metal carbide | 75 to 85  |
| Cobalt                   | 5 to 20   |
| Silver                   | .25 to 5  |
| (D)                      |           |
| Refractory metal carbide | 70 to 85  |
| Cobalt                   | 25 to 5   |
| Silver                   | 5 to 24.9 |

The preferred contact composition, particularly for applications on engines where vibration is severe, is:

|                  | Per cent |
|------------------|----------|
| (1)              |          |
| Tungsten carbide | 90       |
| Cobalt           | 8        |
| Silver           | 2        |

Other specific compositions which may be mentioned are:

|                    | Per cent |
|--------------------|----------|
|                    | (2)      |
| Tungsten carbide   | 85       |
| Cobalt             | 12       |
| Silver             | 3        |
|                    | (3)      |
| Tungsten carbide   | 75       |
| Cobalt             | 2        |
| Silver             | 23       |
|                    | (4)      |
| Tungsten carbide   | 60       |
| Titanium carbide   | 25       |
| Cobalt             | 6        |
| Silver             | 9        |
|                    | (5)      |
| Molybdenum carbide | 92       |
| Cobalt             | 4        |
| Silver             | 4        |
|                    | (6)      |
| Tungsten carbide   | 45       |
| Tantalum carbide   | 45       |
| Cobalt             | 8        |
| Silver             | 2        |

The preferred method of making the contacts comprises mixing the metal powders together, pressing the powder mixture to form a pressed metal body and then sintering the pressed powder body at an elevated temperature. All the powders used are preferably of -325 mesh fineness and may, for example, have the following average particle size:

|                  | Microns |
|------------------|---------|
| Tungsten carbide | 1.5     |
| Cobalt           | 3 to 5  |
| Silver           | 10      |

It is preferred to mix the tungsten carbide, or other refractory carbide and cobalt powders together first and ball mill them for a considerable period of time, such as 48 hours. This promotes the production of cobalt envelopes surrounding the tungsten carbide particles. The silver powder may then be added and the mixture ball milled again for several more hours, such as 12 hours. It is advisable to add a small amount of a volatile binder such as 1 or 2% glyptal at this stage to promote bonding of the powder mixture. The mixture may then be pressed in a suitable die to form a pressed powder body. A suitable pressed density is 8 grams per c. c. for the preferred composition (1) given above.

The pressed body may then be presintered in hydrogen at 850° C. for one hour and then cut or dressed to suitable dimensions, allowing for further shrinkage to take place on further sintering. A final sintering in pure dry hydrogen at a temperature between 1350° C. and 1500° C. is then given to the body in a closed carbon boat or tube. The preferred sintering temperature is 1450° C. The sintered pellets of composition (1) may have a density around 13.9 grams per c. c. and a hardness around 85-90 Rockwell A.

It will be appreciated that these physical properties are given by way of example only and that the properties of the finished product may be varied depending on the materials and procedures used.

For compositions where the higher silver contents are used, it may be possible in some cases to press and sinter the mixture of refractory metal carbide and cobalt with or without part of the silver to form a sintered porous body and then to heat the body in contact with molten

silver to impregnate the remaining pores with silver.

Where operation at extreme temperatures must be provided for, it is of some considerable importance to attach the refractory carbide contact to a backing having substantially the same low co-efficient of expansion over a comparatively wide range of temperatures.

Materials of low co-efficient of expansion which are suitable are Invar, 30 to 45% nickel steels, alloys such as Kovar or Fernico containing 28% nickel, 18% cobalt, balance iron; materials such as Fernichrome containing 37% iron, 30% nickel, 25% cobalt and 8% chromium, also straight iron-chromium alloys.

Referring to the drawing, Figures 1 and 2 show a contact assembly comprising a facing disc 18 formed of the sintered refractory carbide composition described herein attached to an Invar or other low expansion alloy backing rivet 12 by a thin layer 11 of brazing solder, such as silver solder, pure copper or a copper-nickel alloy. The backing rivet has a shank portion 13 to enable it to be attached to a support in the electrical apparatus in which the contact is used.

Figures 3 and 4 show a button-type contact having a plane facing disc 20 secured by braze 21 to a thin flat disc 22 of backing metal, such as steel, Monel, nickel, bronze or nickel-silver or, where thermal stresses are to be kept low, of Invar or other low expansion alloy. Disc 22 is provided on its back face with a small central rounded dome projection 23 which enables it to be resistance welded to a support such as a leaf spring or other contact arm by clamping the contact and arm between welding electrodes and passing electric current through the junction to melt the projection and cause welding to the contact arm.

Figures 5 and 6 show another contact button wherein the facing disc 30 of the refractory carbide composition has a rounded face.

Figures 7, 8 and 9 show a contact adapted for resistance welding comprising a refractory facing disc 40 having a plane contact face and a concave under side. Backing 42 is a concavo-convex disc, the convex side of which fits into the concave side of disc 40 and is joined to it by brazing solder 41. The contact can be secured to a support by resistance welding wherein rim 43 around the concave depression is backing 42 is fused to the support.

Figures 10 and 11 show a screw type contact and the use of a stress equalizing layer to isolate expansion stresses in the screw backing from the contact face. The assembly comprises refractory composition contact face disc 50 secured by a braze layer 51 to a stress equilizing disc 52 which may be of a non-brittle low expansion alloy, such as Invar or one of the other alloys mentioned. Disc 52 is in turn secured by brazing solder layer 53 to the backing screw 54 which may be of relatively high expansion metal such as steel, brass, bronze or the like. Disc 52 prevents the expansion stresses from the backing screw from being transmitted to the relatively brittle contact facing disc.

Instead of making disc 52 of low expansion alloy, it may be formed of a highly ductile metal or alloy, such as soft silver or copper, which yields sufficiently to absorb thermal stresses.

In comparison tests in an accelerated wear test machine, designed to produce contact abrasion, it was found that the preferred material for the present invention formed of 90% tungsten

carbide, 8% cobalt and 2% silver, had a contact resistance after 396 hours of operation of only .12 ohm and showed a material loss for the moving contact of .0030 gm. and for the stationary contact of .0003 gm., as compared with a contact resistance of 3.15 ohms and a material loss of .0414 gm. for the moving contact and .0348 gm. for the stationary contact both formed of a high commercial grade of tungsten contact material after only 120 hours of operation. Another high grade tungsten contact material developed a contact resistance of 4.15 ohms and a material loss of .0350 gm. from the moving contact and .0370 gm. from the stationary contact after 120 hours of operation. Of twenty different types of contact materials tested none of them exhibited the same advantageous combination of low contact resistance and low material loss of the preferred material of the present invention.

While specific embodiments of the invention have been described, it is intended to cover the invention broadly within the spirit and scope of the appended claims.

What is claimed is:

1. An electric contact suitable for operation under conditions of strong vibration formed of a metal composition of 85 to 95% of a refractory metal carbide selected from the group consisting of tungsten carbide, molybdenum carbide, titanium carbide, zirconium carbide, vanadium carbide, columbium carbide and tantalum carbide, from 2 to 10% cobalt and 0.5 to 5% silver said contact being characterized by high abrasion resistance and low material loss.

2. An electric contact suitable for operation under conditions of strong vibration formed of a metal composition of 87 to 93% tungsten carbide, 6 to 10% cobalt and 1 to 3% silver said contact being characterized by high abrasion resistance and low material loss.

3. An electric contact suitable for operation under conditions of strong vibration formed of a metal composition of 90% tungsten carbide, 8% cobalt and 2% silver said contact being characterized by high abrasion resistance and low material loss.

15

FRANZ R. HENSEL.  
EARL I. LARSEN.  
EARL F. SWAZY.

#### REFERENCES CITED

The following references are of record in the file of this patent:

20

#### UNITED STATES PATENTS

| Number    | Name     | Date          |
|-----------|----------|---------------|
| 1,181,742 | Coolidge | May 2, 1916   |
| 1,979,372 | Duhme    | Nov. 6, 1934  |
| 2,049,317 | Pinta    | July 28, 1936 |
| 2,281,446 | Laise    | Apr. 28, 1942 |
| 2,289,708 | Jackson  | July 14, 1942 |
| 2,313,070 | Hensel   | Mar. 9, 1943  |

30

#### FOREIGN PATENTS

| Number  | Country       | Date          |
|---------|---------------|---------------|
| 345,171 | Great Britain | Mar. 19, 1931 |